

# United States Patent Office

2,720,466

Patented Oct. 11, 1955

1

2,720,466

## ASPHALT COMPOSITIONS

Mathew L. Kalinowski, Chicago, Ill., and Frederick H. MacLaren, Munster, Ind., assignors to Standard Oil Company, Chicago, Ill., a corporation of Indiana

No Drawing. Application December 15, 1951,  
Serial No. 261,921

4 Claims. (Cl. 106—271)

This invention pertains to improvements in asphalt compositions and more particularly relates to asphalt compositions having improved hardening resistant properties.

Resistance to undue hardening is an important property requirement of asphalts, particularly penetration grade paving asphalts and in many localities asphalts for paving and other purposes must possess certain specifications which indicate resistance to undue hardening, which property is measured in terms of recovery penetration. In brief, this test measures the penetration of asphalts recovered from finished asphalt pavements or recovered from asphalts which have been subjected to certain specified conditions which normally promote the hardening of asphaltic materials. Since normally the recovery of an asphalt material from a finished pavement may be inconvenient, and does not evaluate the properties of the asphalt prior to paving, a laboratory procedure has been devised for measuring the resistance to hardening in terms of recovery penetration.

The test known as the Detroit recovery test consists of subjecting the asphalt to the so-called Shattuck oxidation test, described in Association of Paving Technologists Proceedings, Technical Sessions, vol. II (1940), pp. 186-203, and subsequently submitting the product from the Shattuck oxidation test to the Abson recovery method, described in A. S. T. M. Proceedings, 1933 (vol. 33), pp. 704-711. In the Shattuck oxidation procedure, 1880 grams standard Ottawa silica sand, heated to 400° F. and 120 grams of asphalt heated to 300° F. are introduced into a pug mixer, heated to an inside temperature of 275° F. to 300° F. and mixed for one minute at 75 R. P. M. The mixture is then removed from the mixer and spread evenly in a straight side shallow metal pan having the dimensions of 7 inches x 11 inches x 1 1/4 inches deep. The pan is immediately placed in a thermostatically controlled electric oven, heated at 350° F. for exactly thirty minutes. The mixture is then removed from the oven, cooled and the asphalt recovered by the Abson method.

The Abson method involves extraction of the asphalt with benzol in a Soxhlet-type extractor, and the solvent removed by distillation in an atmosphere of carbon dioxide. The penetration of the solvent-free recovered asphalt is then determined by A. S. T. M. Method 45-49.

In many localities the specifications for paving asphalts require that the penetration of the asphalt recovered from finished pavements must be at least 50% of the original penetration for resurfacing work and at least 60% of the original penetration for new road work. Asphalts obtained from asphaltic crude oils usually meet the specified recovery penetration. However, asphalts obtained from mixed crude oils containing waxes, such as paraffin waxes, frequently have a recovery penetration of less than 50% and are unsatisfactory with respect to resistance to hardening.

It is an object of the present invention to provide a wax-containing asphalt which will have a recovery penetration of at least 50%. Another object of the invention

2

is to provide a wax-containing penetration grade paving asphalt which is resistant to hardening. A further object of the invention is to provide a method of increasing the resistance to hardening of wax-containing paving asphalts. Still another object of the invention is to provide a method of increasing the recovery penetration of wax-containing paving asphalts to a value of at least 50% of the original penetration of such asphalt. Other objects and advantages will become apparent from the following description thereof.

10 In accordance with the present invention the resistance to hardening characteristics of wax-containing asphalts, particularly penetration grade paving asphalts, is enhanced by incorporating in such asphalts from about 0.1% to about 10%, and preferably from 0.5% to 5% of a condensation product of an aromatic compound and a condensable aliphatic compound having more than 10 carbon atoms. These condensation products are preferably made by Friedel-Crafts condensation of an aromatic compound with a relatively long chain aliphatic compound containing a reactive group, such as a replaceable halogen atom, preferably chlorine atom, or an olefinic linkage, such as for example, chlorinated paraffin wax, chlorinated heavy paraffin oil, chlorinated montan wax, or olefins derived therefrom by the removal of the hydrogen chloride without cracking the C—C linkage. The aromatic compound may be an aromatic hydrocarbon, or various derivatives thereof, such as aromatic hydrocarbons containing low molecular weight alkyl groups, such as methyl, ethyl, etc., or other constituents, such as hydroxy or alkoxy groups, such as for example, benzene, naphthalene, toluene, xylene, diphenyl, phenol, etc. Several materials suitable for use in the present invention for the purpose of improving the resistance to hardening of solid asphaltic materials are available. One such compound is a product known as "Poure," which is a naphthalene-chlorinated paraffin wax condensation product prepared by the methods described in U. S. Patents Nos. 1,963,917, 1,963,918 and 2,057,104. Another product marketed under the trade name, "Paraflo" is made by condensing about 10 to 20 parts by weight of naphthalene with 90 to 80 parts by weight of chlorinated paraffin wax containing about 10 to 15% chlorine in the presence of a Friedel-Crafts catalyst, such as aluminum chloride. Another product marketed by Monsanto Chemical Company under the trade-name "Stanopour" is made by similar condensation of phenol with chlorinated paraffin wax in the presence of aluminum chloride, which product may or may not be further reacted upon with a resinifying agent, such as acyl halides, for example, phthalyl chloride. These condensation products are oil-soluble having molecular weights above 500 and may range as high as 2000 or 5000, or more.

As an example of one method of making the wax condensation products employed in our process, paraffin wax having a melting point of 126° F.-130° F. may be heated with chlorine in a glass lined vessel until the amount of chlorine absorbed by the wax reaches 10% to 15%. The resulting chlorinated wax may then be mixed with about 10% of its weight of naphthalene and to the melted mixture at a temperature of 150° F. to 400° F. there is added, with vigorous agitation, 5% to 10% of anhydrous aluminum chloride. The reaction proceeds rapidly and within 30 minutes the reaction is substantially complete. The reaction mixture is then washed with water and neutralized, a hydrocarbon diluent being added at this stage to facilitate handling the heavy condensation products. A suitable diluent may be naphtha, kerosene or other light hydrocarbon oil. After neutralization it is preferred to remove the diluent by distillation.

The condensation product may be incorporated in the solid asphaltic material by well known and convenient

methods, such as by stirring while the asphaltic material is heated and in a fluid state. Other additives for bituminous materials, such as wet mineral aggregate coating agents, may be incorporated in the asphalt materials containing the condensation products herein described. The present invention is applicable to increasing the resistance to hardening of wax-containing normally liquid asphalts such as road oils, cutbacks, wood treating asphalts, etc., or normally semi-solid or solid asphalts obtained by vacuum and/or steam reduction, including penetration grade paving asphalts, or oxidized wax-containing asphalts, such as roofing asphalts, paper coating asphalts, canal lining asphalts, etc.

Penetration grade wax-containing asphalts or wax-containing asphalt cements are fluxed or unfluxed asphalts having a penetration at 77° F. of between about 5 and 300 under a load of 100 grams applied for five seconds.

The following example illustrates a specific embodiment of the herein described invention. A solid paving asphalt prepared by steam and vacuum reduction of a wax-containing Texas crude oil and a blend of this asphalt containing 0.5% of "Pourex," a condensation product obtained by the aluminum chloride condensation of naphthalene with paraffin wax containing 10%-15% chlorine were subjected to the above described recovery test procedure and the following results obtained:

*Recovery penetration of wax-containing paving asphalt*

| Asphalt                               | Original Penetration | Penetration After Test | Recovery Pen., Percent |
|---------------------------------------|----------------------|------------------------|------------------------|
| (A) Wax-containing West Texas Asphalt | 111                  | 41                     | 37                     |
| (B) A+0.5% "Pourex"                   | 94                   | 57                     | 61                     |

The penetrations were obtained by A. S. T. M. Method D5-49 at 77° F. with a 100 gram load for five seconds. The recovery penetration, percent, is the ratio of the penetration of the asphalt after the test to the original penetration of the asphalt. The resistance to hardening is indicated by the increase in the recovery penetration, expressed in percent.

Percentages given herein and in the appended claims are weight percentages, unless otherwise stated.

It is not intended that this invention be limited to the particular example, which has been given merely for illustration, but only by the appended claims in which it is intended to claim all novelty inherent in the invention as well as other modifications coming within the scope and spirit of the invention.

We claim:

1. A paving asphalt composition having improved resistance towards hardening, comprising a major proportion of a wax-containing paving asphalt normally susceptible to hardening, and from 0.1% to about 10% of an aluminum chloride condensation product of an aromatic hydrocarbon and a chlorinated paraffin wax.

2. A paving asphalt composition having a recovery penetration of at least about 50%, comprising a major proportion of a wax-containing paving asphalt normally having a recovery penetration of less than about 50%, and from 0.1% to about 10% of an oil-soluble aluminum chloride condensation product of naphthalene and a chlorinated paraffin wax containing from about 10% to about 15% chlorine.

3. An asphalt cement composition having improved resistance to hardening comprising a major proportion of a wax-containing asphalt cement normally susceptible to hardening and from about 0.1% to about 10% of an aluminum chloride condensation product of an aromatic hydrocarbon and a chlorinated paraffin wax.

4. An asphalt composition comprising a major proportion of a wax-containing asphalt and from 0.1% to about 10% of a condensation product of an aromatic compound selected from the class consisting of an aromatic hydrocarbon and a phenol and a chlorinated paraffin wax, said condensation being carried out in the presence of a Friedel-Crafts catalyst.

*References Cited in the file of this patent*

UNITED STATES PATENTS

|           |               |               |
|-----------|---------------|---------------|
| 2,085,373 | Loane         | June 29, 1937 |
| 2,191,295 | Dohse         | Feb. 20, 1940 |
| 2,248,749 | Engelhardt    | July 8, 1941  |
| 2,429,565 | Reiff         | Oct. 21, 1947 |
| 2,465,960 | Berge         | Mar. 29, 1949 |
| 2,492,848 | Crouch et al. | Dec. 27, 1949 |